

## UNITED STATES PATENT OFFICE

2,378,305

## STABILIZATION OF COLORING COMPOSITIONS CONTAINING DIAZONIUM SALTS

Hans Z. Lecher, Plainfield, and William B. Hardy and Frederic H. Adams, Bound Brook, N. J., assignors to American Cyanamid Company, New York, N. Y., a corporation of Maine

No Drawing. Application July 5, 1943,  
Serial No. 493,594

13 Claims. (Cl. 8—71)

This invention relates to compositions containing diazonium salts derived from ice color diazo components and to methods of preventing the thinning of printing pastes containing such diazo compounds.

An important method of producing prints of azoic colors on vegetable fibers consists in padding the goods with an alkaline solution of an azoic coupling component and printing these goods with a printing paste containing a diazonium salt derived from an ice color diazo component. The diazonium salt is either prepared by the printer himself by diazotizing the corresponding base or it is applied in the form of a stable diazonium salt. This simple and well-known cheap process is open to a very serious disadvantage. The printing pastes containing the diazonium salts and a carbohydrate thickener tend to thin out rapidly losing their desired printing consistency. It is with this thinning action that the present invention is concerned.

According to the present invention the diazonium salt is associated with a water soluble sulfonic acid containing at least one olefinic double bond or acetylenic triple bond for each 10 carbon atoms.

When an aromatic amine is diazotized in acid solution, a diazonium salt is formed which is generally assumed to have the following formula:



where Ar stands for the aromatic radical of the diazo component and X stands for the anion of the acid. These diazonium salts are salts of the very strong diazonium bases and the aqueous solutions contain essentially the diazonium cations and the anions of the acid used, as indicated by the formula. Some of these diazonium salts are difficult to isolate because of their great solubility. Others are not so soluble and can be easily isolated. Some are difficult to handle after isolation because of their explosivity, others are rather stable and do not represent an explosive hazard. It is also known that if the anion of the

acid X<sup>-</sup> is properly chosen, in almost all cases diazonium salts of lower solubility may be produced and therefore isolated, and it is also known that many of these diazonium salts have lost their explosive character and can be stored and handled in the dry state without danger; this kind of diazonium salts is sometimes referred to as "stabilized" diazonium salts. They comprise such compounds as certain aromatic sulfonates, without olefinic double bonds, borofluorides; and particularly salts of complex acids sometimes referred to as double salts, the most important of them being the double salts of diazonium chlorides and zinc chloride which correspond to the formula:



It should be borne in mind that also these "stabilized" diazonium salts including the above mentioned double salts are true diazonium salts, i. e., the aqueous solution contains the same diazonium cations as the solution of any other diazonium salt derived from the same base. The stabilized diazonium salts should not be confused with other kinds of stabilized diazo compounds such as diazotates, also known as nitrosamines, or diazoamino and diazoimino compounds which are only stable and applied in alkaline medium, while on the other hand the diazonium salts are only stable applied in acid medium. The present invention deals with inhibiting the thinning action of diazonium salts only and not with any similar action that might be observed with other types of diazo compounds. Whenever stabilized diazo compounds are referred to in this application this term shall be interpreted to include exclusively stabilized diazonium salts and not to include diazotates or diazoamino or diazoimino compounds.

While it is not intended to limit the present invention to any theory of action, we believe that it is highly probable that lowering of viscosity of printing gums is essentially caused by the diazonium cation because the same kind of thing

results regardless of the anion of the diazonium salt and even the double salts of the stabilized diazonium salts described above exert a similar thinning action. Presumably in aqueous solution the stabilized diazonium salts are ionized to give the same diazonium cation. The pH of the printing paste is not critical so long as it is on the acid side, for the present invention does not deal with any other types of pastes. Alkaline media, as is well-known, cause rearrangement of the diazonium salts to diazo compounds of different structure which are referred to as diazotates or nitrosamines.

While not desiring to limit the invention thereto, we believe that the evidence strongly indicates that the thinning action is a colloidal phenomenon rather than a chemical reaction. The following test was made: A diazonium salt derived from 2-nitro-4-methoxy aniline was added to a printing paste made up with a starch thickener; after 20 hours the then water thin solution was coupled with an alkaline solution of beta-naphthol and the azo dye formed was removed by filtration. The amount of azo dyestuff obtained indicated that the bulk of the diazonium salt was undecomposed and had acted while the filtrate still showed the reaction of starch and not the reactions of reducing sugars.

The thinning action differs widely and depends upon the structure of the diazo component the diazonium salt derives from. We have found that those diazonium salts that are known to be very active couplers are also the worst thinners, while those that are slow in coupling generally thin to a much lesser degree. Though there is certainly some parallelism in the coupling power and thinning action these two properties are not strictly proportionate. The diazonium salts that derive from nitroanilines are the worst thinners. Particularly those deriving from 2,4-dinitro-6-chloroaniline, from 2-nitro-4-chloroaniline, from 2-nitro-4-methoxy aniline, from 2-nitro-4-methylaniline thin the vegetable gums very badly. The diazonium salts deriving from o-nitraniline thin more than those deriving from the meta and para compounds. On the other hand the diazonium salts deriving from the 2-methyl-4-chloroaniline and from o-anisidine have only little thinning action. Obviously, the rate of the thinning depends upon the concentration of the diazonium ions present in the printing paste.

The thinning action has been observed with all thickeners prepared from materials of vegetable origin such as starches, gums, alkyl celluloses, etc. Wheat starch, corn starch, rice starch, sweet potato starch, tapioca starch, chlorinated starch, may be mentioned as examples of starches. Carob bean gum and gum tragacanth may be mentioned as examples of gums and methyl- or ethyl-cellulose as examples of alkyl celluloses. Obviously, also mixtures of these materials are quite often used in thickeners and their viscosity is equally influenced by diazonium salts. It will be noted all of these thickeners are carbohydrates or carbohydrate derivatives. In the claims the expression "carbohydrate thickener" is used in a broad sense to cover pure carbohydrates and derivatives.

The water soluble sulfonic acids containing at least one olefinic double bond or acetylenic triple bond for each 10 carbon atoms have the general property of preventing or reducing the thinning action of diazonium salts on printing pastes. The precise mechanism of the thinning action of in-

hibitors is not yet fully determined but without wishing to limit the invention to any theory of action, the following hypothesis is presented as a probable explanation.

We believe that the diazonium cations which are the active thinning agents are unsaturated and have a marked tendency to combine. This unsaturated character is probably responsible for the ease with which they combine with coupling components to form azo dyestuffs. When an unsaturated thinning inhibitor such as an unsaturated sulfonic acid is added to the diazonium salt solution before the printing thickener is added, it is probable that the diazonium cation forms a loose complex with the thinning inhibitor which decreases the affinity of the diazonium cation and inhibits its action upon the thickener. When the thickener is first added to the diazonium salt solution followed by addition of the thinning inhibitor, thinning is prevented to a much lesser degree. Apparently in such a case the diazonium salt has already commenced its thinning action on the thickener and the action is not reversible so that the addition of the thinning inhibitor does not remedy the damage already done.

The present invention includes all the diazonium salts derived from ice color diazo components, that is to say, from all diazotizable aromatic amines free from solubilizing groups useful in making ice colors or azoic pigments. Typical are the following:

Aniline and its homologues, as e. g. the toluidines, 2,4-dimethylaniline; halogen derivatives of aniline and of its homologues, as e. g. the mono-fluoroanilines, the monochloroanilines, 2,5-difluoroaniline, 2-fluoro-5-chloroaniline, 2,5-dichloroaniline, m - aminobenzotrifluoride, p - aminobenzotrifluoride, 3 - amino-4 - chlorobenzotrifluoride, 2-methyl-3-chloroaniline, 2-methyl-4-chloroaniline, 2-methyl-5-chloroaniline, 3-methyl-4-chloroaniline, 5-methyl-2-chloroaniline, 2-methyl - 4 - chloro - 5 - bromoaniline, 2-methyl-4,5-dichloroaniline, 4-methyl-2,5-dichloroaniline; nitro derivatives of aniline and of its homologues and their halogen derivatives, as e. g. the nitroanilines, 2-methyl-4-nitroaniline, 2-methyl-5-nitroaniline, 4-methyl-2-nitroaniline, 2-nitro-4-fluoroaniline, 2-nitro-4-chloroaniline, 3-nitro-4-chloroaniline, 4-nitro-2-chloroaniline; ether derivatives of primary aromatic amines and their halogen derivatives, as e. g. o-anisidine, 2-methoxy-5-methyl aniline, 2,5-dimethoxy-aniline, 2-methoxy-1-naphthylamine, 2-amino-diphenylether, 2-amino-4-acetyl-diphenylether, benzyl-2-aminophenyl-ether, 3-fluoro-4-methoxyaniline, 2-methoxy-5-chloroaniline, 2,5-dimethoxy-4-chloroaniline, 2-methoxy-4-chloro-5-methyl aniline, 2-methoxy - 5 - bromoaniline, 3-bromo-6-ethoxyaniline, 4-chloro-2-amino-diphenylether, 4-amino - 2 - chloro-diphenylether, 4-amino-4-chlorodiphenylether, 4,4'-dichloro - 2 - amino - diphenylether, 2,2',5',5'-trichloro-4-amino-diphenylether; ether derivatives of aniline and its homologues containing nitro groups as e. g. 2-methoxy-4-nitroaniline, 2-methoxy-5-nitroaniline, 2-nitro-4-methoxyaniline, 2-methoxy-4-nitro-5-methyl-aniline; monoacyl derivatives of aromatic diamines, as e. g. N-hexahydrobenzol-p-phenylene diamine, N-hexahydrobenzoyl - p - toluyl-enediamine, N-benzoyl - p - phenylene diamine; monoacyl derivatives of diaminophenol ethers, as e. g. 2-benzoylamino - 4 - amino - anisole, 2-hexahydrobenzoylamino - 5 - aminoanisole, 2 - amino - 5 - benzoylamino - hydroquinone dimethyl 75 ether and diethylether, 2-amino-5-hexahydro-

benzoylamino-hydroquinone dimethylether and diethylether, 2 - amino - 5 - butyrylamino-hydroquinone dimethylether and diethylether, 2-amino-5 - phenoxyacetylamino - hydroquinone diethylether, the monomethyl and the monobenzyl and the monophenyl-urethane of 2,5-diamino-hydroquinone dimethylether and diethylether, 1-amino-3-benzoylamino-4,6-dimethoxy - benzene; analogous monoacyl derivatives of 2,5-diamino-4-alkoxy-toluenes and of 2,5-diamino-4-alkoxy-chlorobenzenes and of 2,5-diamino-4-alkoxy-benzene sulfodialkylamides; analogous monoacyl derivatives of 1,3-diamino-4,6-dimethylbenzene; the diethylamide of 2-amino-4(4'-chlorophenoxy)-benzoic acid; monoacyl derivatives of diamino-p-chlorophenyl ethers as e. g. 2-amino-4-chloro-5-acetylaminodiphenylether, 2-benzylamino-4-chloro-5-aminoanisole; amino derivatives of aromatic sulfones as e. g. 3-amino-4-methyldiphenyl sulfone, 2-amino-4'-methyl-diphenyl sulfone, 2-amino-4-acetyl-diphenyl sulfone, the ethyl ester of 3-amino-4-(p-toluenesulfonyl)-benzoic acid, 4 - methoxy - 3 - amino-phenyl - ethyl sulfone, (4 - methoxy - 3 - amino-phenyl) - benzyl sulfone, 4-ethoxy-3-amino-diphenyl sulfone, 2 - amino - 4 - (trifluoromethyl) - phenyl-ethyl sulfone; amino derivatives of aromatic dialkylsulfonamides as e. g. 3-amino-4-methyl-benzene dimethylsulfonamide and diethylsulfonamide, 3-amino - 4 - methoxy-benzene diethylsulfonamide; xenylamine; alpha and beta naphthylamine; alpha aminoanthraquinone; 2-amino-3-nitro-fluorene and 2-amino - 3 - nitro-fluorenone; amino-diarylamines and their ether derivatives and their nitro derivatives as e. g. 2-methoxy-5-amino-diphenylamine, 4-methoxy-4'-amino-diphenylamine, 4 - ethoxy - 4' - amino-diphenylamine, 3,4'-dinitro - 4 - amino-diphenylamine; amino-azo compounds, as e. g. 3,2'-dimethyl-4-amino-azobenzene, 2-methyl-4-amino-5 - methoxy-4'-chloroazobenzene, 4-amino-4'-nitro-3-methoxy-6-methyl-azobenzene, 4 - amino - 4'-nitro-2,5-dimethoxy-azobenzene, 4-amino-4'-chloro-3-methoxy-6-methyl-azobenzene, the azo dye; diazotized o-anisidine coupled onto alpha naphthylamine.

There are also diazonium salts deriving from aromatic diamines in which only one of the amino groups is diazotized and they also fall within the scope of the present invention. An example of this type of amine is 2,6-dichloro-1,4-phenylene diamine. Diazonium salts deriving from diamines in which both amino groups are diazotized to form tetrazo compounds fall within its scope. Typical amines of this class are p-phenylene diamine, benzedine, o-tolidine, o-dianisidine, 4,4'-diamino stilbene, 4,4'-diamino diphenylamine, 2,2'-dimethyl-4,4'-diamino diphenylamine and 1,5-diamino naphthalene.

Also diazonium salts deriving from heterocyclic amines or diamines fall under the present invention. Typical heterocyclic amines are 2-amino-carbazole, 3,6-diaminocarbazole, 2-nitro-3-amino-carbazole, 2 - nitro - 3-aminodibenzofuran, 2-amino-3-nitrobenzothiophene, 1 - amino-5-fluorobenzothiazole:



Obviously also mixtures of different diazonium salts may be used.

The inhibitors useful in the present invention

include the water soluble sulfonic acids that contain at least one olefinic double bond or acetylenic triple bond. The inhibitors of the present invention may contain one or more olefinic double bonds or acetylenic triple bonds in the same molecule, or they may contain both double bonds and triple bonds. We have found that the anti-thinning action appears to depend mainly on the presence of the double or triple bond. In order to be practically effective, we have found that there must be a certain minimum number of the unsaturated bonds in a molecule of given size. Practically useful anti-thinning action is obtained when there is at least one double bond or triple bond per 10 carbon atoms of the molecule of the sulfonic acid. The unsaturated bond may be located almost anywhere in the molecule. Thus, it may be linked directly to the carbon to which the sulfonic acid group is connected or it may be located elsewhere in a carbon chain, which may be interrupted by other elements such as oxygen, nitrogen, sulfur and the like.

The sulfonic acid compounds used in the present invention are true sulfonic acids or sulfonates, that is to say organic compounds containing the group  $\equiv C - SO_3H$ , and it is necessary that the inhibitor be free from groups which are capable of azoic coupling with the diazo compound or condensation to form a diazoamino or diazoimino compound in acid medium. It is also necessary that the cation of the inhibitor shall not be capable of coupling with the diazo compound, condensing therewith to form a diazoamino or diazoimino body or of catalytically decomposing it as is the case with certain copper compounds. The present invention is not limited to using a single inhibitor and mixtures are equally effective. Since the sulfonic acid compounds stabilize in an aqueous composition the acid itself or its water soluble salts may be used.

Examples of aliphatic sulfonic acids containing one double bond are: ethylene sulfonic acid, 2-propene-1-sulfonic acid, 2-methyl-2-propene-1-sulfonic acid, 2-butene-1-sulfonic acid, 1,1-dimethyl-2-propene-1-sulfonic acid, 3,3-diethyl-2-propene-1-sulfonic acid. Examples of aliphatic sulfonic acids containing two double bonds are: 1,6-heptadiene-4-sulfonic acid, 3,7-dimethyl-2,6-octadiene-1-sulfonic acid. As an example of an aliphatic sulfonic acid with a triple bond there may be mentioned 2-propene-1-sulfonic acid. With the exception of ethylene sulfonic acid these aliphatic sulfonic acids are most conveniently prepared by reacting the corresponding chloride with sodium sulfite in the well-known manner.

The unsaturated grouping does not necessarily have to be connected to the sulfonic group by a carbon chain. On the contrary this chain may be interrupted by other atoms. Typical examples are N-allyl taurine, diallyl sulfosuccinate, and dimethylallyl sulfosuccinate, a compound containing 12 carbon atoms and two olefinic double bonds. The latter two compounds may be obtained from the corresponding maleic acid esters by reaction with sodium bisulfite.

The sulfonic acids of the present invention need not belong to the aliphatic series. On the contrary they may contain ring systems, so long as there is at least one olefinic double bond or a triple bond. It should be noted that the double bond must be olefinic in nature, thus for example the double bonds in the benzene ring are not olefinic in nature and accordingly benzene sulfonic acid does not behave as an inhibitor and is not included in the present invention. How-

ever, alicyclic compounds which do contain double bonds of olefinic character are active inhibitors. Typical examples are cyclohexene-3-sulfonic acid, 1-p-menthene-8-sulfonic acid and 1-p-menthene-4-sulfonic acid which are obtainable from the corresponding chlorides.

While the ordinary sulfonic acids of the aromatic series are not included in the present invention because the aromatic rings do not contain double bonds of olefinic character, it should be noted that the presence of an aromatic ring in the molecule does not affect its inhibiting action provided that the molecule also contains olefinic double bonds or acetylenic triple bonds outside of the aromatic ring. Typical examples of such compounds as styrene-beta-sulfonic acid, alpha-methylstyrene-p-sulfonic acid, phenyl acetylene-p-sulfonic acid, and the like.

As with the purely aliphatic compounds referred to above, the sulfonic group does not have to be connected to the unsaturated group through a carbon chain only. Thus for example the allyl ether of phenol p-sulfonic acid acts as inhibitor.

Heterocyclic sulfonic acids are also useable as long as they contain double bonds or triple bonds of olefinic or acetylenic character respectively. These bonds may be inside or outside of the heterocyclic rings.

Inhibitors of the present invention may have other substituent groups, thus for example allyl ethers of 2-sulfo-4-nitrophenol, 2-sulfo-4-chlorophenol, or 2-sulfo-4-aminophenol are useful inhibitors.

It should be noted however, that the inhibiting effectiveness is not unaffected by the presence of substituents. The so-called negative substituents when attached directly to a carbon of the double bond group lower the inhibiting action. Thus ethylene sulfonic acid is by no means as powerful an inhibitor as 2-propene-1-sulfonic acid where the negative group is separated from the double bond by a methylene group. This behavior appears to be general with the sulfonic acids of the present invention and is further evidence that the double or triple bond is the portion of the molecule which apparently exerts the primary inhibiting action.

Since the sulfonic acids of the present invention behave as they do by reason of their anion and their effectiveness is not greatly influenced by the nature of the cation except where it interferes as in the case of copper, it is preferable in many cases to use a salt of the sulfonic acid instead of the sulfonic acid itself as these salts may be very readily handled.

The sodium and potassium salts of the sulfonic acids of the present invention are the cheapest ones and in general the most convenient to prepare. The invention, however, is not in any sense limited to the use of these preferred salts and on the contrary other salts such as zinc or calcium salts may be used. Ammonium salts and salts of organic bases such as amines, amidines, guanidines and the like may be used.

The inhibitors of the present invention may be added in two stages, either before or after the diazotization. In the first place the aromatic bases known as ice color diazo components may be blended with the inhibitor and such blends may be subsequently diazotized in the customary manner and incorporated into a printing paste. The equivalent of this procedure is to dissolve the inhibitor and the base separately before the dia-

zotization. If the inhibitors are used in this manner they obviously should not contain diazotizable amino groups. In the second place diazonium salts either stable per se or stabilized in a customary way, may be blended with the inhibitor to form solid compositions suitable for incorporation into printing pastes. The obvious equivalent is to add the inhibitor to a separately prepared diazo solution before the printing paste is made up. It does not make any difference what procedure is used in every case the thinning of the printing gum is greatly delayed.

If the diazonium salt is first mixed with the printing gum and the inhibitor is added afterwards, then in a great many cases of very active diazo compounds a certain amount of thinning has already taken place before the inhibitor is added. This procedure, therefore, should be used only where the thinning action is slow, but it is included in the broad scope of the invention.

The invention will be further illustrated with the specific examples which describe typical embodiments of the present invention. The parts are by weight.

#### Example 1

Four parts of a mixture of the zinc chloride double salt of the diazonium chloride obtained from 3-nitro-4-amino anisole, and of partially dehydrated magnesium sulfate, this mixture containing 25.3% of that amine in the diazotized form, and 0.288 part of sodium-2-propene-1-sulfonate of the following formula:



are dissolved in 21 parts of water and the resulting solution is thoroughly mixed with 75 parts of a 2½% carob bean gum. The resulting paste is suitable for use in the production of fast color prints on textile material, especially cotton cloth, impregnated with ice color coupling components such as the anilide of 2-hydroxy-3-naphthoic acid, bis-acetoacetic-o-tolidide, etc. The advantage of a printing paste such as this over one made in a similar manner, but without the sulfonate is shown in the following table:

| Printing gum used                                    | Relative viscosity measurement after two minutes | Relative viscosity measurement after two hours |
|------------------------------------------------------|--------------------------------------------------|------------------------------------------------|
| Printing gum containing sodium-2-propene-1-sulfonate | 40.7                                             | 17.3                                           |
| Same, but without sodium allyl sulfonate             | 41.4                                             | 1.3                                            |

The relative viscosity is expressed by the times in seconds taken for copper plated steel shot weighing approximately 0.107 gram each to fall through 130 millimeters of the printing paste.

#### Example 2

In a manner similar to that described in Example 1 printing pastes are made containing the zinc chloride double salts of the diazonium chlorides of the following ice color bases, sodium-2-methyl-2-propene sulfonate of the following formula:



and suitable thickening gums. In every case

the sulfonate inhibits the thinning of the printing paste as is shown in the following table:

ice color coupling components. The superiority of a printing paste thus made over one similarly

| Base used for the preparation of diazo | Diluent of stabilized diazo | Stabilized diazo used corresponds to parts real base | Parts real sodium-2-methyl-2-propene-1-sulfonate used | Water used, parts | Kind and percent of gum used (75 parts) | Viscosity measurement 2 min. after mixing | Time of second reading after mixing | Second viscosity measurement | Method of measurement of relative viscosity |
|----------------------------------------|-----------------------------|------------------------------------------------------|-------------------------------------------------------|-------------------|-----------------------------------------|-------------------------------------------|-------------------------------------|------------------------------|---------------------------------------------|
| 3-nitro-4-amino anisole.               | Magnesium sulfate.          | 0.74                                                 | 0.106                                                 | 21                | Carob bean 2.5%--                       | 70.5                                      | Hours 2                             | 34.3                         | A1                                          |
| Do.....                                | do.....                     | 0.74                                                 | 0                                                     | 21                | do.....                                 | 73.0                                      | 2                                   | 0.9                          | A1                                          |
| 4-nitro-2-amino anisole.               | 0.....                      | 0.84                                                 | 0.106                                                 | 25                | do.....                                 | 47.2                                      | 3                                   | 33.4                         | A1                                          |
| Do.....                                | 0.....                      | 0.84                                                 | 0                                                     | 25                | do.....                                 | 46.0                                      | 3                                   | 15.4                         | A1                                          |
| 2,5-dichloroaniline.                   | 0.....                      | 0.81                                                 | 0.106                                                 | 21                | do.....                                 | 56.6                                      | 3                                   | 37.7                         | A1                                          |
| Do.....                                | 0.....                      | 0.81                                                 | 0                                                     | 21                | do.....                                 | 53.6                                      | 3                                   | 5.0                          | A1                                          |
| 3-nitro-4-amino anisole.               | 0.....                      | 0.84                                                 | 0.273                                                 | 21                | Methyl cellulose (methocel 4000) 3%     | 40.5                                      | 21                                  | 23.4                         | A3                                          |
| Do.....                                | 0.....                      | 0.84                                                 | 0                                                     | 21                | do.....                                 | 40.5                                      | 21                                  | 7.2                          | A3                                          |
| Dianisidine                            | 0.....                      | 0.61                                                 | 0.106                                                 | 21                | Carob bean 2.5%--                       | 19.3                                      | 2                                   | 13.6                         | A2                                          |
| Do.....                                | 0.....                      | 0.61                                                 | 0                                                     | 21                | do.....                                 | 20.0                                      | 2                                   | 6.3                          | A2                                          |

<sup>1</sup> Note.—On viscosity measurements: A1 Cu plated steel shot weighing .353 g. dropped 130 mm., time in seconds. A2 Cu plated steel shot weighing .107 g. dropped 130 mm., time in seconds. A3 glass spherical beads .097 g. dropped 130 mm., time in seconds.

### Example 3

An intimate mixture is made of 100 parts of 3-nitro-4-amino anisole, 25 parts of sodium-2-methyl-2-propene-1-sulfonate of approximately 73% purity, and 75 grams of sodium chloride. This mixture can be treated with mineral acid and sodium nitrite and the resulting diazo solution can then be buffered with sodium acetate and mixed with thickening gum for the production of fast color prints on textile materials impregnated with ice color coupling components such as arylides of 2-hydroxy-3-naphthoic acid, etc.

Printing pastes made from such mixtures have the advantage over those pastes made from the ordinary bases unblended with inhibitors in that the gums made from the blended bases retain their viscosity much longer than the others. This advantage can best be seen by consulting the following table. In this table the change of viscosity of printing pastes containing various diazos and sodium-2-methyl-2-propene-1-sulfonate as inhibitor is compared with the change of viscosity of similar pastes containing no inhibitor. In each case the base, or mixture of base with inhibitor, is treated with hydrochloric acid and sodium nitrite in the usual manner:

prepared but without the sulfonate is shown by the following figures:

| 30 | Printing paste used | Relative viscosity measurement after $\frac{1}{2}$ hour | Relative viscosity measurement after $3\frac{1}{2}$ hours |
|----|---------------------|---------------------------------------------------------|-----------------------------------------------------------|
|    |                     | Gum containing inhibitor.....                           | Same but without inhibitor.....                           |
|    |                     | 15.2                                                    | 10.3                                                      |
|    |                     | 13.4                                                    | 2.3                                                       |

The viscosity measurements indicated above are the times in seconds for lead shot weighing 0.069 gram each to fall 130 millimeters.

### Example 5

5.03 parts of the zinc chloride double salt obtained from diazotized 3-nitro-4-amino anisole corresponding to 16.7% real base are mixed with 0.408 part of the allyl ether of sodium p-phenol sulfonate. This mixture is dissolved in 21 parts of water and the resulting solution is intimately mixed with 75 parts of 2.5% carob bean gum. The superiority of a printing paste thus made

| Base diazotized          | Parts of 73% sodium-2-methyl-2-propene-1-sulfonate per part base | Inert diluent and parts per part base | Parts real base in gum | (75 parts) gum used and strength | Viscosity reading 2 min. after mixing | Time of second viscosity measurement after mixing | Second viscosity reading | Method of viscosity measurement |
|--------------------------|------------------------------------------------------------------|---------------------------------------|------------------------|----------------------------------|---------------------------------------|---------------------------------------------------|--------------------------|---------------------------------|
| 5-nitro-2-amino anisole  | 0.5                                                              | Sodium chloride 0.5                   | 0.84                   | Carob Bean 2.5%--                | 25.3                                  | Hours 4                                           | 13.2                     | A2                              |
| Do.....                  | 0                                                                | 0                                     | 0.84                   | do.....                          | 22.2                                  | 4                                                 | 4.2                      | A2                              |
| 4-chloro-2-nitro-aniline | 0.94                                                             | 0                                     | 0.69                   | do.....                          | 27.0                                  | 4                                                 | 13.5                     | A2                              |
| Do.....                  | 0                                                                | 0                                     | 0.69                   | do.....                          | 24.1                                  | 4                                                 | 0.8                      | A2                              |

### Example 4

1.58 parts of a product containing the zinc chloride double salt obtained from tetrazotized o-dianisidine corresponding to 48.8% of real base and 0.215 part of potassium 2-methyl-2-propene-1-sulfonate of 70% purity are intimately mixed and dissolved in 23 parts of water and the resulting solution is thoroughly mixed with 75 parts of 2% carob bean gum. This viscous paste is useful for the preparation of deep blue patterns upon cellulosic material impregnated with arylides of 2-hydroxy-3-naphthoic acid, or other

over one similarly prepared, but without inhibitor is shown in the following table:

| 65 | Printing paste used | Relative viscosity measurement after 5 minutes | Relative viscosity measurement after 4 hours |
|----|---------------------|------------------------------------------------|----------------------------------------------|
|    |                     | Paste containing inhibitor.....                | Paste without inhibitor.....                 |
|    |                     | 60.2                                           | 29.8                                         |
|    |                     | 47.0                                           | 0.7                                          |

These relative viscosity measurements are the times in seconds for copper plated steel shot weighing 0.107 gram each to fall 130 millimeters.

## Example 6

1.79 parts of the zinc chloride double salt obtained from diazotized 3-nitro-4-amino anisole corresponding to 47% real base are mixed with 0.35 part of ammonium styrene beta-sulfonate and the resulting mixture is dissolved in a mixture of 20 parts of water and 1 part of 5N hydrochloric acid. This solution is intimately mixed with 75 parts of 2.5% carob bean gum. The advantage of the printing paste thus prepared over one made similarly but without the inhibitor is shown in the following table:

| Printing paste used        | Relative viscosity after 2 minutes | Relative viscosity after 4 hours |
|----------------------------|------------------------------------|----------------------------------|
| Paste containing inhibitor | 153.1                              | 43.4                             |
| Paste without inhibitor    | 147.3                              | 1.0                              |

These relative viscosity measurements are the times in seconds for spherical glass beads weighing 0.097 gram to fall 130 millimeters.

As can be seen styrene beta-sulfonate is a less effective inhibitor because of the proximity of the double bond and of the sulfonic group.

This application is in part a continuation of our co-pending application, Serial No. 437,224, filed April 1, 1942.

We claim:

1. Diazo compositions suitable for printing, containing a water soluble diazonium salt derived from an ice color diazo component and an organic compound having not more than 12 carbon atoms belonging to the group consisting of water soluble sulfonic acids containing at least one olefinic double bond for each 10 carbon atoms, water soluble sulfonic acids containing at least one acetylenic triple bond for 10 carbon atoms, and water soluble salts of the above acids, the sulfonic acid compounds being free from constituents capable of azoic coupling with the diazonium salt, catalytic decomposition thereof at room temperature or condensation therewith to form diazoamine or diazoimino compounds in acid medium, the amount of the sulfonic acid compound being sufficient to substantially inhibit thinning of a carbohydrate thickener.

2. A printing paste containing a carbohydrate thickener, at least one water soluble diazonium salt derived from an ice color diazo component and an organic compound having not more than 12 carbon atoms belonging to the group consisting of water soluble sulfonic acids containing at least one olefinic double bond for 10 carbon atoms, water soluble sulfonic acids containing at least one acetylenic triple bond for each 10 carbon atoms, and water soluble salts of the above acids, the sulfonic acid compound being free from constituents capable of azoic coupling with the diazonium compound, catalytically decomposing the same at room temperature or condensation therewith to produce diazoamine or diazoimino compounds in acid medium, the amount of the

sulfonic acid compound being sufficient to substantially inhibit thinning of the carbohydrate thickener.

3. A composition according to claim 1 in which the diazonium salt is a diazonium chloride-zinc chloride double salt.

4. A composition according to claim 2 in which the diazonium salt is a diazonium chloride-zinc chloride double salt.

10 5. A diazo composition comprising a water soluble diazonium salt derived from 3-nitro-4-amino anisole and a sufficient amount of sodium 2-methyl-2-propene-1-sulfonate to substantially inhibit thinning of a carbohydrate printing thickener by the diazonium salt.

6. A printing paste containing a carbohydrate thickener and a water soluble diazonium salt derived from diazotized 3-nitro-4-amino-anisole and a sufficient amount of sodium 2-methyl-2-propene-1-sulfonate to substantially inhibit thinning of the paste.

7. A composition suitable for the preparation of printing pastes containing carbohydrate gum thickeners comprising an ice color forming component included in the group consisting of compositions containing water soluble diazonium salts and intermediates therefor consisting of amines diazotizable to produce compositions containing water soluble diazonium salts, the color forming component having associated therewith an organic compound with not more than 12 carbon atoms selected from the group consisting of water soluble sulfonic acids containing at least one olefinic double bond for each 10 carbon atoms,

25 35 water soluble sulfonic acids containing at least one acetylenic triple bond for each 10 carbon atoms, and water soluble salts of the above acids, the sulfonic acid compounds being free from constituents capable of azoic coupling with the diazonium salt, catalytic decomposition thereof at room temperature, or condensation therewith to form diazo amino or diazo imino compounds in acid medium, the amount of sulfonic acid compound being sufficient to substantially inhibit thinning of a carbohydrate thickener.

45 8. A composition according to claim 7 in which the thinning inhibitor is the sodium salt of 2-methyl-2-propene-1-sulfonic acid.

9. A composition according to claim 1 in which the thinning inhibitor is the sodium salt of 2-methyl-2-propene-1-sulfonic acid.

10. A composition according to claim 3 in which the thinning inhibitor is 2-methyl-2-propene-1-sulfonic acid.

55 11. A composition according to claim 7 in which the thinning inhibitor is N-allyl taurine.

12. A composition according to claim 1 in which the thinning inhibitor is N-allyl taurine.

13. A composition according to claim 3 in which the thinning inhibitor is N-allyl taurine.

HANS Z. LECHER.  
WILLIAM B. HARDY.  
FREDERIC H. ADAMS.